

June 7, 1927.

1,631,423

A. LUCAS

METHOD OF PURIFYING IRON SCALE

Filed May 16, 1925



INVENTOR

*Anton Lucas.*  
BY  
*Arthur C. Brown*  
ATTORNEY

Patented June 7, 1927.

1,631,423

# UNITED STATES PATENT OFFICE.

ANTON LUCAS, OF KANSAS CITY, MISSOURI.

## METHOD OF PURIFYING IRON SCALE.

Application filed November 16, 1925. Serial No. 69,333.

My invention relates to a method of purifying iron scale as a step in the manufacture of an aluminothermic mixture, of a character particularly adapted for use in 5 welding car rails and making heavy repairs, as of iron or steel beams, girders or the like, the principal object of the invention being the separation of sand, dirt or other foreign matter from the scale, to provide a mechanically 10 pure product and insure against variability in chemical reaction due to unbalanced oxide content in the mixture.

A mixture of the character described consists of calcined ferroso-ferric oxide and a 15 powder of aluminum or other metal or alloy capable of reducing the oxide. For convenience, only aluminum will be hereinafter mentioned as the reducing agent, with the understanding that other metals or alloys 20 capable of performing the reduction may be employed as well, without departing from the invention.

While oxide desirable for the machine may be secured from different sources, as 25 from magnetic iron stone or other ore, the most convenient source and that capable of producing the purest oxide is the iron scale from rolling or like mills. In such mills the scale has heretofore been considered a 30 by-product which, accumulating in somewhat large quantities, has been fed back to the blast furnace as an addition to the charge, but considered of inferior value, partly because of its impurities, principally 35 mechanical, due to the presence with the scale of mill dust and frequently small pieces of iron. Scale of this kind before mixture with the aluminum element is calcined or roasted, preferably with an oxidizing 40 flame to drive off any liquid content or chemical impurities, oxidize any particles of iron present with the scale, and make the oxygen content uniform.

When so treated the roasted product is 45 screened, and in some instances attempt is made to separate the scale from its impurities by magnetic treatment. I have found, however, that screening or sifting is ineffectual, as any mesh coarse enough to pass the scale flakes or particles will also pass solid impurities such as sand, brick or iron particles of such size and in sufficient quantities to affect reaction in the reducing 50 crucible. The scale flake is quite brittle and 55 may be pulverized in a crusher under a

pressure which will not affect the harder particles constituting the impurities.

I have, therefore, added to the customary process of purifying the scale, a mechanical step consisting of crushing the scale between relatively soft rollers, having sufficient tension to pulverize the scale, but yieldable to the harder particles, and then separating the product by air blast or fine screening or both.

The accompanying drawing illustrates a form of crusher which may be employed for the purpose, consisting of rubber or like rolls 1, on shafts 2, journaled in a frame 3, one yieldably and the other fixedly, and driven by a belt 4 to rotate the rollers in the opposite directions and feed the mixture therethrough as in an ordinary mangle. The material may be fed to the rolls from a hopper 5 and cascaded from the rolls 75 through an air blast, indicated by 6, onto a screen 7.

The loose roller is urged to contact with the fixed one by springs 8, sufficiently strong to press and crush the scale, but yieldable to allow the loose roller to spread upon the passage of an excessively large solid particle therethrough, the material of which the rolls are composed being sufficiently soft to embed the usual run of hard material during 85 the feeding travel.

The drawing also illustrates the material and the method of treatment, 9 designating the material coming to the crusher, comprising the scale flakes and commingled impurities, 10 a piece of brick, sand, iron or other hard material embedded in the soft rollers, 11, light dirt and dust separated from the heavier particles by the air blast, 12 the pure pulverized iron scale which is passed 95 through the fine screen to be collected in a storage receptacle and 13 the heavier impurities which have been rejected by the screen.

I have found that by so treating the iron 100 scale I eliminate impurities which, if allowed to remain in the scale, would upon the reaction produce gases that would remain in the solidified metal, causing blow holes and other defects, and a much more effective 105 material may be produced with which a surer and more effective weld may be made.

Inasmuch as mixture of the purified scale with proper reducing agents and the method of use of the mixture is well known, I 110

will not describe the same in detail, as neither the generic mixture, the welding process nor any specific apparatus for crushing the scale is claimed as my invention, the 5 invention including only the method of treating the scale for purification.

What I claim and desire to secure by Letters-Patent is:—

1. The method of purifying iron scale, 10 consisting of crushing the scale between crushing elements yieldable to substances of greater hardness than the scale and then separating the light crushed substances

from the other substances, and then separating the scale from the remaining substances. 15

2. The method of purifying iron scale, consisting of passing mill scale between feeding rolls of a material sufficiently resistant to crush the scale, but yieldable to substances less brittle than the scale, and then separating the light crushed substances from the heavy scale and the hard materials and then screening the crushed scale from the hard material gravitationally. 20

In testimony whereof I affix my signature.  
ANTON LUCAS.